

## 1

2,872,356

**LUBRICATION OF SYNTHETIC CELLULOSE FIBERS**

Harry W. Bull, Midland, and Walter A. Finke, Saginaw, Mich., assignors to The Dow Chemical Company, Midland, Mich., a corporation of Delaware

No Drawing. Application June 2, 1955  
Serial No. 512,852

3 Claims. (Cl. 117—139.5)

This invention relates to the sewing of synthetic cellulosic fibers.

It has long been known that the needles of commercial sewing machines frequently become hot during operation at high speeds. Consequently thermoplastic threads such as those of synthetic cellulosic fibers soften during sewing. Under these conditions the least stoppage may cause the filaments to fuse together in the eye of a needle with the resultant breaking of the thread when the sewing is resumed or the speed is increased. It has also been found that the action of the needle tends to cut thermoplastic threads thereby causing injury to the fabric.

Attempts to alleviate this difficulty have previously been made with organic dressings such as waxes, mineral oils, vegetable oils and the like. It has been found, however, that many of these heretofore employed thread dressings tend to dissolve synthetic fibers and therefore appreciably reduce their strength. This is particularly true of yarns composed of synthetic cellulosic materials. Furthermore yarns which have been treated with these conventional lubricants have little or no protection against the heat developed in the needle of the machine.

It is the object of this invention to provide a treatment for synthetic cellulosic fibers which will enable them to be satisfactorily sewn. Other objects and advantages will be apparent from the following description.

This invention relates to a sewing thread composed of synthetic cellulosic fibers, which have been impregnated with a fluid diorganopolysiloxane in which the organic radicals are monovalent hydrocarbon radicals attached to the silicon atom through silicon-carbon linkages.

It has been found that threads coated with these fluid organopolysiloxanes can be sewn with ease without any appreciable reduction in the tensile strength of the fibers. This invention makes possible the commercial sewing of ethyl cellulose threads which heretofore could not be satisfactorily sewn on commercial machines even when treated with conventional organic thread coating materials.

The organopolysiloxanes operative in this invention are any fluid monovalent hydrocarbon substituted siloxane. Suitable examples of such siloxanes are those of the unit formula  $R_2SiO$  or  $R_3SiO_{0.5}$  and copolymers of these siloxanes. The fluids may also contain monoorganopolysiloxane units and  $SiO_2$  units.

For the purpose of this invention the hydrocarbon radicals on the silicon can be any monovalent hydrocarbon radical such as alkyl radicals such as methyl, ethyl and octadecyl; alkenyl radicals such as vinyl, allyl or hexenyl; cycloaliphatic hydrocarbon radicals such as cyclohexyl or cyclohexenyl; aryl hydrocarbon radicals such as phenyl, tolyl, xenyl and naphthyl; and aralkyl hydrocarbon radicals such as benzyl.

Any synthetic cellulosic fiber is included within the scope of this invention. These include, for example, cellulose ethers such as methyl cellulose, ethyl cellulose, propyl cellulose and benzyl cellulose; cellulose esters such as cellulose acetate, cellulose propionate and cellulose butyrate and regenerated cellulose.

## 2

The organopolysiloxane may be applied to the fibers in any convenient manner. The precise mode of application will depend largely upon the nature of the material and the use for which it is intended. In general, the thread dressing or lubricant may be applied by any of the standard procedures such as by dipping, padding or spraying. It is frequently advantageous to apply the siloxane to the thread in solution of an organic solvent such as petroleum ether, toluene, benzene and the like.

For the purpose of this invention the viscosity of the siloxane is not critical and it may range from thin fluids to soluble gums.

The following examples are illustrative only and should not be construed as limiting the invention which is properly delineated in the appended claims.

*Example 1*

A liquid dimethylsiloxane polymer having a viscosity of 5,200 cs. at 25° C. was dissolved in an equal weight of petroleum ether. Ethyl cellulose thread of 1,800 denier yarn was passed through the solution and then wiped on felt to remove the excess liquid. The thread was wound on a cone and was used to sew filter bags made of ethyl cellulose twill woven cloth. The sewing machine operated satisfactorily at a speed of 2,000 to 3,000 stitches per minute. In contrast, ethyl cellulose thread of the same construction which had been coated with a vegetable base lubricant, fused and broke readily on the same machine operated at a speed of 1,000 to 1,500 stitches per minute.

Portions of the above thread were tested for tensile strength. The thread coated with the dimethylsiloxane polymer showed no loss in tensile strength at the end of two or three days storage at room temperature. By contrast the thread coated with the vegetable base lubricant had lost three pounds in tensile strength after storage at room temperature for two to three days.

*Example 2*

Ethyl cellulose thread similar in quality to that employed in Example 1 was coated with a liquid dimethylsiloxane having a viscosity of 302 cs. at 25° C. The excess liquid was removed by wiping with felt and the coated thread was tested for abrasion resistance as follows: The thread was wound (3/4 wrap) on a 1/16 inch diameter polished wire and then pulled with a six inch stroke back and forth around the wire at a tension of 500 grams. The number of strokes required to break the thread was determined.

The siloxane coated thread ran for 59 strokes. By contrast an identical type thread coated with a commercial vegetable spinning oil broke after 38 strokes under identical test conditions.

*Example 3*

Improved sewing is obtained when the following fluid siloxanes are employed in the procedure of Example 1: phenylmethylsiloxane, ethylmethylsiloxane, octadecylmethylsiloxane, vinylmethylsiloxane, vinylphenylsiloxane, copolymers of dimethylsiloxane and trimethylsiloxane, copolymers of diethylsiloxane, monomethylsiloxane and phenyldimethylsiloxane and copolymers of trimethylsiloxane and  $SiO_2$ .

*Example 4*

Improved sewing qualities are obtained when cellulose acetate threads are treated in accordance with the procedure of Example 1.

That which is claimed is:

1. A sewing thread composed of synthetic cellulosic fibers, said thread being coated with a fluid organopoly-

siloxane in which the organic radicals are monovalent hydrocarbon radicals, said thread being more resistant to infusion breaks and more easily sewn than similar threads of the same composition which have not been treated with the siloxane.

2. A sewing thread in accordance with claim 1 wherein the siloxane is a methylsiloxane.

3. A sewing thread composed of fibers of ethyl cellulose coated with a methylpolysiloxane fluid.

## References Cited in the file of this patent

## UNITED STATES PATENTS

|   |           |                  |               |
|---|-----------|------------------|---------------|
| 5 | 2,494,513 | Kropscott et al. | Jan. 10, 1950 |
|   | 2,524,895 | Dodge            | Oct. 10, 1950 |
|   | 2,637,623 | Janes            | May 5, 1953   |
|   | 2,698,817 | Guenther         | Jan. 4, 1955  |